

Feb. 26, 1929.

1,703,636

G. C. RASCH

RUG AND METHOD OF MAKING THE SAME

Filed Nov. 22, 1926

FIG. 1



FIG. 2



FIG. 3



Inventor  
Gustave C. Rasch,  
By Frank E. Demmett,  
Atty.

Patented Feb. 26, 1929.

1,703,636

# UNITED STATES PATENT OFFICE.

GUSTAVE C. RASCH, OF BURLINGTON, WISCONSIN, ASSIGNOR TO BURLINGTON BLANKET COMPANY, OF BURLINGTON, WISCONSIN, A CORPORATION OF WISCONSIN.

## RUG AND METHOD OF MAKING THE SAME.

Application filed November 22, 1926. Serial No. 149,891.

This invention relates to rugs and method of making the same, and the object of the invention is to improve the construction and texture of rugs in the manner to be herein-  
5 after described and claimed.

Referring to the drawings, which accompany this specification and form a part here-  
10 of, which drawings illustrate an embodiment  
of this invention, and on which drawings the  
same reference characters are used to design-  
ate the same parts wherever they may ap-  
pear in each of the several views, Fig. 1 is a  
15 perspective view of a rug; Fig. 2 is a partial  
section, on a greatly enlarged scale, on the  
line 2—2, on Fig. 1, looking in the direction  
indicated by the arrows; and Fig. 3 is a sec-  
tion similar to Fig. 2, but on a smaller scale,  
20 and also showing component parts of the rug  
separated and illustrating the method of mak-  
ing the same.

Referring to the drawings, the reference  
numeral 1 designates a rug, which, as illus-  
trated by the drawings, is composed of differ-  
25 ent layers of materials. The reference numer-  
al 2 designates a stay for the bottom of the rug  
which may be of any suitable material. The  
drawings illustrate the stay 2 as composed  
30 of burlap which is a suitable material for the  
stay 2. The reference numeral 3 designates  
a filling layer, or cushion, of loosely matted  
fibers, as distinguished from a felt. In mak-  
ing the rug, the rug is built up from the bot-  
35 tom by first needling the filling layer or cushion  
3 after the filling layer or cushion 3 has  
been placed upon the stay 2. This first nee-  
dling operation, which may be performed by  
means of an ordinary needling machine, not  
40 only needles the matted fibers composing the  
filling layer or cushion 3 together, but also  
needles, or anchors this filling layer 3 to the  
stay 2. The result of the first needling op-  
eration is illustrated at 9 in Figure 3 of the  
45 drawing. The filling layer 3 may be composed  
of comparatively cheap grades of wool with  
which animal hair or bristles or any suitable  
animal or vegetable fibers may be mixed. An  
upper stay 4 is then placed on top of the fill-  
50 ing layer or cushion 3 and this upper stay 4 is  
treated with glue or sizing or any other suit-  
able adhesive material. This treatment of the  
upper stay 4 with an adhesive material may  
be readily and economically performed by  
running a suitable material, preferably a  
55 woven material, through a liquid bath of  
adhesive and squeezing out excess adhesive

by a roll or rolls, for example to leave the stay  
sized with an adhesive, but moist for succeed-  
ing needling operations. An upper layer of  
loosely matted fibers, a bat of wool, for ex-  
ample, 5 is then placed on top of the upper 60  
stay 4 and the rug, as thus far completed, is  
subjected to another needling operation, while  
the upper stay 4 is still moist with the adhe-  
sive. The result of a second needling opera-  
tion is illustrated at 10 in Figure 3 of the 65  
drawing. This needling operation not only  
needles the fibers of the upper layer 5 to-  
gether but carries fibers from the upper layer  
5 down through the moist upper stay 4 and  
into the filling layer or cushion 3. The nee- 70  
dling, referred to, is usually performed in ma-  
chines which have a large number of needles  
pointing downward and with barbs project-  
ing from the needles and extending towards  
the points of the needles. This needling opera- 75  
tion may be such that the needles and their  
lowermost barbs run entirely through the fill-  
ing layer or cushion 3 and the bottom stay 2,  
or, if desired, the lowermost barbs of the nee-  
dles, which are the mechanical means for 80  
catching and carrying fibers with them, may  
not be permitted to pass through the lower  
stay 2. A finishing layer 6, preferably of a  
nice grade of wool, may then be needled to the  
upper layer 5 and, preferably, this needling 85  
operation is performed while the upper stay 4  
is still moist and the lower barbs of the nee-  
dles are, preferably, forced through not only  
the upper layer 5 but also through the upper  
stay 4 while the upper stay 4 is still moist 90  
with the adhesive. The finishing layer 6 is  
provided, as a separate layer, to provide the  
rug with a surface of a better quality of ma-  
terial than that used for the filling layer or  
cushion 3 and the upper layer 5. The finish- 95  
ing layer 6 also provides an easy method for  
imparting designs or ornamentations to the  
top of the rug as will be readily understood  
from an inspection of Fig. 1 of the drawings  
which illustrates a rug with its body part 7 of 100  
a substantially general uniform appearance  
with a contrasting border 8. Fig. 1 of the  
drawings merely illustrates an example of or-  
namentation of the top of the rug and the  
ornamentation is, of course, subject to practi- 105  
cally an infinite number of variations.

By needling layers of a rug together with  
an interposed sized stay, the needling opera-  
tions being performed while the sized stay  
is still moist, a rug is produced in which 110

parts are not only needled together but enough fibers are also cemented together to give the rug, when dried, a stiffness and substantiality which prevents the rug from curling at its corners and edges and prevents it from being easily scuffed and wrinkled.

It will be understood, of course, that the separation of the stays and the layers, as shown by Fig. 3 of the drawings, is only intended to emphasize the relationship of the parts of the rug to each other.

I have referred to my invention as an improvement in rugs and method of making the same for the reason that the completed fabric is used extensively for coverings for floors and the like under the common and popular use of the term "rug," but I wish it to be understood that I have used the term "rug" in a broad sense to designate a fabricated material which may be used in any place and under any conditions for which it is suited.

What I claim is:

1. The process of making rugs, which consists in needling a layer of matted fibers through a stay, moistened with an adhesive, into another layer of matted fibers, while the adhesive on the stay is still moist.
2. The process of making rugs which consists in needling a layer of matted fibers, imposing thereon a stay moistened with an adhesive, imposing on the stay another layer of loosely matted fibers, and needling said

last mentioned layer of fibers through the stay, while still moist with the adhesive, into the first mentioned layer of matted fibers.

35

3. A rug composed of two layers of matted fibers with a stay impregnated with an adhesive therebetween, with the layers needled together through the stay and fibers of both layers cemented to the stay and to each other.

40

4. A rug composed of a bottom stay, a filling layer or cushion of loosely matted fibers needled together and anchored to said bottom stay, an adhesive impregnated stay and an upper layer of loosely matted fibers needled together and through said upper stay and to said filling layer or cushion with fibers of the filling layer or cushion and the upper layer cemented to said upper stay and to each other.

45

5. A rug composed of a bottom stay, a filling layer or cushion of loosely matted fibers needled together and anchored to said bottom stay, an adhesive impregnated stay, an upper layer of loosely matted fibers needled together and through said upper stay and to said filling layer or cushion with fibers of the filling layer or cushion and the upper layer cemented to said upper stay and to each other, and a finishing layer needled on top of the rug.

55

In witness whereof I hereto affix my signature.

GUSTAVE C. RASCH.

60